

R. A. HADFIELD, A. G. MCK. JACK AND I. B. MILNE.  
ARMOR PIERCING PROJECTILE.  
APPLICATION FILED OCT. 4, 1918.

1,381,633.

Patented June 14, 1921.



Inventors:  
Sir Robert A. Hadfield  
Alexander G. Mck. Jack  
Isaac B. Milne

By

J. Rosehill Ward,  
Attorney

# UNITED STATES PATENT OFFICE.

ROBERT ABBOTT HADFIELD, OF WESTMINSTER, ALEXANDER GEORGE MCKENZIE JACK, OF SHEFFIELD, AND ISAAC BERNARD MILNE, OF TOTLEY, ENGLAND.

## ARMOR-PIERCING PROJECTILE.

1,381,633.

Specification of Letters Patent. Patented June 14, 1921.

Application filed October 4, 1918. Serial No. 256,890.

To all whom it may concern:

Be it known that we, Sir ROBERT ABBOTT HADFIELD, Bart. F. R. S., ALEXANDER GEORGE MCKENZIE JACK, and ISAAC BERNARD MILNE, subjects of the King of Great Britain and Ireland, residing, respectively, at Westminster, England, Sheffield, in the county of York, England, and Totley, in the county of Derby, England, have invented 5 Improvements in or Relating to Armor-Piercing Projectiles, of which the following is a specification.

This invention relates to the manufacture of armor piercing projectiles or shells of all 15 calibers, particularly of large diameter, say of twelve inches and upward, designed to perforate thick hard faced armor plates without becoming broken up, or broken to such an extent as to interfere with their subsequent desired action.

For this purpose in the specification of another application for Letters Patent filed 28th June 1915, Serial No. 36886, there are described processes for the production of 25 such a projectile made of nickel-chromium steel, according to which the projectile, after being formed to shape, as by casting it solid and then, after suitably annealing it, pressing it to shape in a suitable press, is hardened 30 by heating it all over in a suitable furnace to a hardening temperature, and then dipping it directly point downward to its base end in a cooling medium properly to cool and harden it. The projectile thus hardened 35 all over is then tempered by heating its base portion to a suitable tempering temperature in a tempering furnace while its pointed end portion is immersed, point downward, to a suitable depth in water, after which it is 40 partially cooled and the whole shell then cooled in a suitable cooling medium.

According to one example described in the said former specification, carried out with a twelve inch projectile having a length of 45 about thirty four inches and made of nickel-chromium steel having the following approximate composition, namely, carbon .6 to .7%, nickel 2 to 3%, and chromium 2 to 3%, for example, carbon about .66%, nickel about 50 2.52% and chromium about 2.31%, the projectile was heated all over to a hardening temperature while its point was protected from direct contact with the heat, so that the external shoulder portion of the shell had a temperature of about 55 915° C., to 920°

C., the inner surface of core adjacent to the shoulder portion being found to have, in the example given, a temperature of about 900° C. to 905° C., the point a temperature of about 890° C. and the base a temperature 60 of about 780° C. The projectile thus heated was then hardened all over by dipping it in oil, as the cooling medium, to its base end and holding it there until properly hardened, the cooling being effected from the 65 exterior alone, that is to say without admitting any cooling medium to the interior of the shell. The hardened projectile was afterward subjected to a second or tempering treatment consisting in heating its base 70 or body portion in a furnace to a temperature of about 670° to 705° C., its interior or core having a temperature of about 605° C. while its pointed end portion was immersed 75 to a depth of about eight and a half inches in water kept cold. It was then allowed to cool down in the furnace to a base or body temperature of about 320° C. to 300° C., and an internal or core temperature of about 290° to 255° C. whereupon it was quenched 80 outright in water. When thus treated, the pointed portion of the shell for about the first ten inches of its length has a ball hardness of 600 and over, the weight of this portion comprising about 12% of the total 85 weight of the projectile, the ball hardness varying from 600 at ten inches from the point to 418 at fourteen inches, 311 at eighteen inches and 241 at the base end of the shell. 90

According to a second example, carried out with a fourteen inch projectile having a length of about fifty two inches and made of nickel-chromium steel having the following approximate composition, viz., carbon 95 .69, nickel 2.53% and chromium 2.70%, the projectile was heated all over, while its point was protected from direct contact with the heat, so that the external shoulder portion of the shell had a temperature of about 930° C., the inner surface or core adjacent to the shoulder being found to have in this example a temperature of about 900° to 905° C., the point a temperature of about 875° C., and the base a temperature of about 100 850° C. The projectile thus heated was then dipped in oil to its base end and held in that position until practically cold, the cooling 105 being effected wholly from the exterior inward. The hardened projectile was after 110

ward subjected to a second or tempering treatment consisting in heating the base portion to a temperature of about 700° C., its interior or core having a temperature of about 630° C. while its point was immersed for about a depth of eight inches in water kept cold. The shell was then allowed to cool down in the furnace to a base temperature of about 310° C. and a core temperature of about 255° C. and then quenched outright in water. In this case the pointed end portion of the shell for about the first eight inches of its length had a ball hardness of 652 and over, this portion constituting about 15 6% of the weight of the shell, the hardness decreasing to the base where it was about 262.

In this way there is obtained an armor piercing shell the head or ogival forward portion of which is of different degrees of hardness, varying say from a ball hardness of from about 600 to 700 at the pointed front end portion or zone through successive rearward zones of about 500, 400 and 300 ball hardness, the zone having a ball hardness of about 400 terminating rearwardly, say around about the forward portion of the core or cavity in the shell and the zone having a ball hardness of about 300 extending farther rearward to a lower ball hardness than 300.

The degree of hardness corresponding to a ball hardness of 600 and above is herein-after referred to for brevity and distinction as A ball hardness, the degrees of ball hardness corresponding to 500 to 600 is herein-after referred to as B ball hardness, that corresponding to 400 to 500 as C ball hardness, that corresponding to 300 to 400 as D ball hardness and that below 300 as E ball hardness.

Now the present invention has for its object, better to adapt armor piercing projectiles produced according to the invention described in the former specification to successfully withstand, when suitably capped, the stresses to which they are subjected when striking a hard faced armor plate, particularly under certain special conditions, namely, at comparatively low velocities and 50 at considerable angles and such as obtain for instance in long range firing.

For the purpose mentioned, an armor piercing projectile, formed of nickel-chromium steel of suitable composition, is heated, 55 hardened and tempered in such a manner that the zones of steel of A, B, C, D and E ball hardness in the ogival shaped head of the projectile are moved forward relatively to those of the particular projectiles mentioned in the said former specification, so that there is a much less volume or percentage of steel of A ball hardness than was previously the case and so that steel of E ball hardness extends approximately from a 60 point corresponding to or slightly rearward

of the junction of the ogive and parallel portion of the body of the projectile to the base of the projectile and so that the steel composing the successive zones of B, C, D and E ball hardness, or some of them, shall have imparted to them a high tensile strength with a high elastic limit, a high degree of toughness, a high degree of elongation and high compressive strength or stiffness, in order that such zones shall be 75 adapted better to resist fracture and to support the hardened front end portion of A ball hardness than heretofore under the firing conditions of comparatively low velocity and large striking angle hereinbefore mentioned.

To enable these characteristics to be obtained, a projectile formed of nickel-chromium steel containing say from about .58 to .69% of carbon, from about 2 to 3.5% of nickel and from about 2 to 3% of chromium is heated all over to a less degree than in the examples described in our former specification, say to a hardening temperature of about 800 to 860° C. and then dipped point downward to base in a cooling medium consisting in this case of water, wherein it is allowed to remain until properly hardened, when it is removed from the quenching bath.

The projectile thus hardened all over is tempered by heating it to a base temperature of about 760° C. and an internal temperature of about 575° to 700° C. at a point corresponding to the junction of the head with the body of the projectile, while the head portion is immersed point downward to a comparatively small depth in water to obtain the desired result, after which the projectile is cooled down in the tempering plant to an internal or core temperature of the order of say about 320° C. to 120° C. and then withdrawn from the tempering furnace and cooled, it may be by quenching it outright in a cooling liquid, for example water, or by dipping it point downward in a cooling liquid, for example water, to a suitable zone depth, or it may be allowed to cool slowly in air, or it may be cooled down to atmospheric temperature before removal from the tempering plant.

The duration of the tempering treatment, the depth to which the head portion of the projectile is immersed in water during such treatment and the mode of finally cooling the tempered projectile can be varied and depends to some extent upon the size of the projectile and also upon the percentage of steel in the zones of steel having A, B, C, D and E ball hardness desired.

In all cases, the tempering treatment is such that the percentage of the zone of steel of A ball hardness in the head of the projectile shall be small. The zone of A ball hardness is disposed at the forward end or

nose of the projectile and together with the succeeding zones B, C and D are in the form of shallow or flattened cups arranged one behind the other and extending more 5 or less transversely, as indicated approximately by the dotted lines  $a$  and  $a'$  in the drawing the rearward zone of E ball hardness extending throughout the body of the projectile to the base end thereof. Zones of 10 hardness of the type mentioned are herein referred to for brevity as transverse hardness. Such type of hardness is obtained by immersing the head of the hardened projectile in water to a depth up to say 15 about 2 to 5 inches for say a fourteen inch projectile. The proportions and positions of the different zones of A, B, C, D and E ball hardness can be varied as may be required and according to the type of attack 20 desired, by varying the depth of immersion of the head of the hardened projectiles during the tempering treatment.

Satisfactory results have been obtained with a percentage of A ball hardness of the 25 order of about .25 to 2% of the total weight of the projectile, of B ball hardness of the order of about 2 to 6% of C ball hardness of the order of about 5 to 10% of D ball hardness of the order of about 14 to 20%, the remainder of the projectile being of E ball hardness and extending from around about and over the forward end of the core or chamber of the projectile to the base of the projectile.

To enable the tempering of hardened 30 projectiles to be successfully carried out in a readily controllable manner and so as to enable a number of projectiles having uniform characteristics to be obtained, the tempering of the projectile may advantageously be effected in the manner and by the means described in the specification of another application for Letters Patent filed 27th June, 1914, Serial No. 847680.

According to one example, a hardened and 35 tempered projectile having a diameter of 13.5 inches and which gave satisfactory results under test, was made of nickel-chromium steel containing about .65% of carbon, 2.64% of nickel and 2.6% of chromium and 40 hardened at a temperature of about 820° to 830° C. by dipping it point downward to its base end into water where it was allowed to remain until properly hardened and then removed.

The projectile thus hardened all over was 45 then subjected to the tempering process. For this purpose the body and base portion of the projectile was heated in a suitable tempering furnace, such as that hereinbefore referred to, externally to a temperature of the order of about 760° C. at the base and internally to a temperature of the order of about 660° C. at the forward end of the core, while the head portion of the projectile was immersed point downward to a

zone depth of about three and one half inches in water during the tempering treatment. When the body and base of the projectile had been heated externally and internally to about the temperature mentioned, 70 they were allowed to cool down in the tempering plant to an internal or core temperature of about 120° C. and then the projectile was removed from the tempering furnace. 75

The toughened wall or body of the projectile at a point 17" from the base had an elastic limit of 41 tons to the square inch and a tensile strength of 50 tons with 17% elongation and 33% reduction in area at the 80 break. At the base the elastic limit of the steel was 35 tons, the ultimate strength 49 tons, the elongation 21% and reduction in area 36%. The steel at the forward end of the core had a ball hardness of about 85 250. The zones A, B, C, and D ball hardness were of the type herein referred to as transverse hardness.

In another example, a 15 inch projectile 90 of nickel chromium steel containing .64% carbon, 2.72% Ni. and 2.75% Cr., was heated externally to about 840° C. at the shoulder and point, 835° C. at the base and to an internal or core temperature of 820 to 825° C.; it was then dipped in water to base until properly hardened. It was afterward tempered by heating the base and body portion externally to a base temperature of about 765° C. and internally to a core temperature of about 660° C. while the point of 100 the projectile was immersed in water, as hereinbefore described. It was afterward cooled while in the tempering furnace to a core temperature of about 120° C. and then removed and quenched. The toughened wall 105 or body of the projectile at a point 19 inches from the base had an elastic limit of 46 tons, a tensile strength of 54 tons, with a 15% elongation and a reduction in area of 31% at the break. At the base the steel had 110 an elastic limit of 41 tons and a tensile strength of 53 tons with 19% elongation and 33% reduction in area at the break. The steel at the forward end of the core had a ball hardness of about 290. In this example 115 the A, B, C, and D zones of ball hardness were also of the type referred to as transverse hardness.

To adapt an armor piercing shell hardened and tempered as described for use, it is 120 provided with a suitable cap, preferably made of a nickel-chromium steel with a hardened front portion.

What we claim is:—

1. The process of hardening an armor 125 piercing projectile made of nickel chromium steel which consists in heating the projectile all over to a hardening temperature of the order of about 800 to 860° C., then dipping it point downward to base in water and al- 130

lowing it to remain there until properly hardened and then removing it from the water.

2. The process of treating an armor piercing projectile made of nickel chromium steel which consists in heating the projectile all over to a hardening temperature of the order of about 800 to 860° C. then dipping it point downward to base in water and allowing it 10 to remain there until properly hardened, then removing it from the water and subsequently subjecting the hardened projectile to a suitable tempering treatment while maintaining its point cool.

15 3. The process of hardening and tempering an armor piercing projectile made of nickel chromium steel which consists in heating the projectile all over to a hardening temperature of the order of about 800 to 860° C., 20 then dipping it point downward to base in water and allowing it to remain there until properly hardened, then heating the hardened projectile to a tempering temperature of the order of about 760° C. while the point 25 of the projectile is immersed to a relatively small depth in a cooling liquid and afterward cooling the projectile.

4. The herein described process of hardening an armor piercing projectile which consists in producing a projectile of the approximate composition of carbon about .58 to .69%, nickel about 2 to 3.5% and chromium about 2 to 3%, heating the projectile all over and dipping it while at a hardening 35 temperature of the order of about 800 to 860° C., point downward to base in water and allowing it to remain there until properly hardened and then removing it.

5. The process of hardening and tempering 40 an armor piercing projectile made of nickel chromium steel which consists in dipping the projectile while at a hardening temperature of the order of about 800 to 860° C. in water so as to harden it all over, allowing it to remain therein until properly hardened, removing the projectile from the water, afterward heating the projectile to a suitable tempering temperature while its pointed end portion is immersed to a relatively small 50 depth in a cooling liquid, and finally cooling the projectile.

6. The process of hardening and tempering an armor piercing projectile made of nickel chromium steel which consists in dipping the projectile, while at a hardening 55 temperature of the order of about 800 to 860° C., point downward to base in water, allowing it to remain there until properly hardened, removing the projectile from the water, afterward heating the projectile to an external temperature of the order of about 760° C. and a core temperature of the order of about 570 to 700° C. at the part 60 corresponding to the junction of the head with the body of the projectile while the head portion of the projectile is immersed

point downward to a comparatively small depth in water, and afterward cooling the projectile.

7. The process of hardening and tempering an armor piercing projectile made of nickel chromium steel which consists in dipping the projectile, while at a hardening temperature of the order of about 800 to 860° C., point downward to base in water, allowing it 75 to remain there until properly hardened, removing the projectile from the water, afterward heating the projectile to an external temperature of the order of about 760° C. and a core temperature of the order of about 80 570 to 700° C. at the part corresponding to the junction of the head with the body of the projectile while the head portion of the projectile is immersed point downward to a comparatively small depth in water, afterward cooling the projectile down to an internal or core temperature of the order of about 85 320 to 120° C. in the tempering furnace, then removing the projectile from the tempering furnace and finally cooling it externally 90 thereto.

8. The process of producing a hardened and tempered nickel chromium steel armor piercing projectile having its head of A, B, C, D and E ball hardness as herein defined, 95 the zone of A ball hardness being disposed at the point of the projectile and the zone of E ball hardness extending approximately from a point corresponding to or slightly rearward of the junction of the ogive and 100 parallel portions of the projectile to the base end of the projectile, which consists in heating the projectile all over and dipping it while at a hardening temperature of the order of about 100 800 to 860° C., point downward to base in water, allowing it to remain 105 there until properly hardened, then removing the projectile from the water and heating it in a tempering furnace to a temperature externally of the order of about 760° 110 C. and internally to a temperature of the order of about 570 to 700° C. at the junction of the head with the body of the projectile while the pointed end portion of the projectile 115 is immersed in water to a depth of from about two to five inches in the case of a fourteen inch projectile, so that the percentage of the zone of steel of A ball hardness at the point of the projectile shall be small, and then cooling the projectile. 120

9. The process of producing a hardened and tempered nickel chromium steel armor piercing projectile having its head of A, B, C, D and E ball hardness as herein defined 125 the zone of A ball hardness being disposed at the point of the projectile and the zone of E ball hardness extending approximately from a point corresponding to or slightly rearward of the junction of the ogive and parallel portions of the projectile to the base 130

end of the projectile, which consists in heating the projectile all over and dipping it while at a hardening temperature of the order of about 800 to 860° C., point downward to 5 base in water, allowing it to remain there until properly hardened, then removing the projectile from the water and heating it in a tempering furnace to a temperature externally of the order of about 760° C. and 10 internally to a temperature of the order of about 570 to 700° C. at the junction of the head with the body of the projectile while the pointed end portion of the projectile is immersed in water to a depth of from about two to five inches in the case of a fourteen <sup>15</sup> inch projectile so that the percentage of the zone of steel of A ball hardness at the point of the projectile shall be small, and then cooling the projectile partly in the tempering furnace and partly externally to such 20 furnace.

Signed at London, England, this nineteenth day of August, 1918.

ROBERT ABBOTT HADFIELD.

ALEXANDER GEORGE MCKENZIE JACK.

ISAAC BERNARD MILNE.